

## UNITED STATES PATENT OFFICE

2,654,670

FLUX FOR TREATING ALUMINUM AND  
ALUMINUM ALLOYS

James A. Davis, Columbus, and La Verne W. Eastwood, Westerville, Ohio, assignors, by mesne assignments, to The Pennsylvania Salt Manufacturing Company

No Drawing. Application April 1, 1950,  
Serial No. 153,486

10 Claims. (Cl. 75—68)

**1** This invention relates to the modification of aluminum or aluminum base alloys and more particularly to a flux composition and method of treating aluminum or aluminum base alloys to improve their physical characteristics.

Aluminum and aluminum base metals in general when cast without prior special treatment are found to have poor grain structure, small pinholes dispersed throughout the metal, poor tensile strength, and to be difficult to work or machine. Also, where the aluminum or aluminum base metal has an appreciable silicon content, poor modification of the silicon in the final casting is observed.

These undesirable characteristics tend to weaken the final metal with respect to its mechanical properties, interfere with later working or machining of the aluminum or aluminum base alloy and, where a fine finish is desired, detract from the appearance of the final finished article, the pinholes producing a dull unattractive porous surface. This results in castings unsuitable for many purposes, e. g. pressure cookers, pistons, household fixtures, etc., thus limiting the useful range of the final cast metal.

Various processes of metal treatment and various treating materials have heretofore been resorted to in order to improve the aluminum or aluminum base alloys in attempts to eliminate or substantially decrease the heretofore mentioned undesirable characteristics found in the final metal castings. However, as far as we are aware, there has been no single process or fluxing material developed, prior to our invention, which will improve the final metal casting obtained with respect to grain structure, pinhole porosity, tensile strength and improved silicon modification. The aluminum treating processes and compositions heretofore used, though frequently giving excellent results with respect to improving the final aluminum casting or sheet metal as to one or maybe two of these characteristics would not benefit the metal treated with respect to the other undesirable characteristics, and would in some instances aggravate these other undesirable characteristics. This is particularly true with respect to grain refiners in general and to silicon modifiers such as sodium metal, their use tending to increase the pinhole porosity of the final cast metal. In addition, the use of sodium metal is hazardous, while the use of a grain refiner such as metallic boron involves an expensive smelting operation. It has, therefore, been necessary, when using prior known treating methods and compositions, to

**2** subject the aluminum being treated to several separate treatments each adapted to improve the final cast metal with respect to a different characteristic.

Among prior materials used for treating aluminum melts can be mentioned boron, titanium, sodium and various gaseous agents including fluorine compounds, these being added to the molten aluminum prior to final casting. Elements such as boron, titanium and sodium were added both in their elemental form and as chemically combined with other elements, the boron and titanium being added mainly for the purpose of improving the grain structure of the final casting, whereas the sodium was found to improve the silicon modification. Gases were generally bubbled through the molten aluminum to help decrease the formation of pinholes in the final casting.

**20** In order to obtain a multiple fluxing action, fluxing ingredients have heretofore been used combining several of the above-mentioned elements into a single flux composition. For example, sodium fluoborate has heretofore been used singly as a fluxing material. However, it has been noted that where such fluxing material has been used alone wholly satisfactory results have not been obtained. Sodium fluoborate, when used alone as a flux material, though tending to improve the physical characteristics of the final castings, is objectionable due to the large amount of dross formed during the fluxing operation. The amount of dross formation is such as to make its use in regular foundry practice substantially prohibitive due to the large amount of metal lost in the dross when the sodium fluoborate is used.

**30** It may be possible to reduce the amount of dross formed by using the sodium fluoborate in smaller amounts and maintaining the temperature of the aluminum or aluminum base metal melt below about 1400° F. However, such operation would be unsatisfactory since it is generally desirable to have a flux which will operate successfully at melt temperatures of about 1400° F. to 1450° F., this being the usual maximum temperature range employed prior to casting.

**40** When attempts were made by us to use sodium fluotitanate alone as a fluxing material for aluminum an increase in pinhole porosity was noted even though the grain refinement and silicon dispersion were at first somewhat improved. The grain refinement obtained, however, apparently was not permanent since the size of the

grains increased appreciably when the metal was later subjected to further melting and casting.

We have now found that if a flux comprising a mixture of an alkali metal fluoborate and an alkali metal fluotitanate, in which at least one of the alkali metals is sodium, is used, instead of using these materials singly, no objectionable amount of dross formation is obtained and the grain structure, pinhole porosity, silicon modification and tensile strength are improved. The resulting aluminum castings, when the aluminum was treated in accordance with our present invention, were found to be particularly improved with respect to grain refinement and tensile strength. In addition, the tensile properties of heat-treatable alloys were not adversely affected by the use of the fluxes but were actually improved. The amount of improvement obtained with respect to any of the above characteristics depended somewhat, as would be expected, on the quality of the melt being treated. It was also noted that the grain size in the final casting was improved by the use of these two materials together as against the improvement obtained where they were used separately.

In practicing our invention the flux composition is preferably prepared by fusing or sintering together the alkali fluoborate and alkali fluotitanate so as to obtain a substantially homogeneous moisture-free flux material. Where the flux is prepared by fusing, the fused flux is preferably poured into small aluminum containers of such size as to contain a measured quantity of the fluxing material, the complete container with flux being inserted into the metal melt when the flux is used. The containers may be sealed so as to prevent the flux becoming contaminated, particularly with moisture, prior to use. However, this precaution is not absolutely necessary since the flux composition shows substantially no tendency to absorb moisture from the air. When the flux composition is prepared by sintering, the sintered material is crushed or ground to the desired particle size and then placed in suitable containers from which measured amounts are used as needed. Where it is desired to have a slow fluxing treatment, it has been found preferable to use the fluxing material in the form of the fused sticks. However where a more rapid fluxing action is required the ground sintered flux is to be preferred. The rate of fluxing action is controlled primarily by the size to which the flux material is reduced in the grinding process.

Satisfactory fluxes may be prepared by using the alkali fluoborate and alkali fluotitanate in varying portions with or without other beneficial fluxing agents added thereto, the final flux composition depending on the particular type of aluminum, scrap, base aluminum, or aluminum metal alloy to be modified. In practice, we have found it preferable, in preparing flux compositions in accordance with our invention, to use from 25 to 75% of sodium fluoborate and 25 to 75% of sodium fluotitanate. Where less than the minimum amounts are used, the beneficial results obtained by using these materials in combination in a fluxing composition is reduced. If more than the upper limits given are used, there is a tendency for the flux composition to show some of the undesirable effects, previously noted as being observed where the alkali fluoborate or the alkali fluotitanate were used alone. In order to better illustrate our invention the following examples of some flux compositions are given. These compositions have been successfully used

in treating various types of aluminum and aluminum metal alloys.

*Example 1*

|                     | Percent |
|---------------------|---------|
| Sodium fluoborate   | 50      |
| Sodium fluotitanate | 50      |

*Example 2*

|                     |    |
|---------------------|----|
| Sodium fluoborate   | 30 |
| Sodium fluotitanate | 30 |
| Calcium fluoride    | 6  |
| Sodium chloride     | 34 |

*Example 3*

|                     |    |
|---------------------|----|
| Sodium fluoborate   | 30 |
| Sodium fluotitanate | 30 |
| Sodium chloride     | 16 |
| Cryolite            | 16 |

*Example 4*

|                     |    |
|---------------------|----|
| Sodium fluoborate   | 30 |
| Sodium fluotitanate | 30 |
| Sodium chloride     | 27 |
| Sodium fluoride     | 13 |

*Example 5*

|                        |    |
|------------------------|----|
| Sodium fluoborate      | 75 |
| Potassium fluotitanate | 25 |

*Example 6*

|                      |    |
|----------------------|----|
| Potassium fluoborate | 50 |
| Sodium fluotitanate  | 50 |

The fluxes in each of the above examples were prepared by fusing together the ingredients listed.

In using flux compositions of our invention, satisfactory results have been obtained when as little as 0.1% by weight of the flux to metal being treated was used. The best results, however, have been observed when 0.2 to 1.0% by weight of the fluxing material was employed depending, among other things, on the size of the melt, larger melts in general requiring smaller percentages of the flux. The flux is inserted within the body of the molten aluminum, preferably near the bottom of the melt, so that gases, such as  $BF_3$ , and other products of decomposition can pass upwards through the molten metal. This can be done by use of a conventional perforated phosphorizer. The flux, after being inserted into the body of the melt, is slowly moved through the melt thus gently stirring the melt as the fluxing action takes place. Too rapid stirring should preferably be avoided since it may, in some instances, actually increase the pinhole porosity of the final casting, particularly where a highly refined aluminum is being treated.

We have found the fluxes of our invention to be more suitably adapted to the treatment of what is commonly known in the trade as secondary metal. However, the invention is in no way limited to such treatment, the beneficial results of our flux treatment being obtained with most aluminum or aluminum base metals, the degree of refinement observed depending somewhat upon the conditions of the aluminum before treatment. In describing our invention several special flux formulations have been given. These formulations are given by way of illustration only in order to better describe the invention and should not be considered in any way as limiting the scope of the invention thereto, it being apparent that many other specific formulations may be prepared which would fall within the teaching of our invention.

Having thus described our invention, we claim:

1. A flux composition for treating aluminum and aluminum base metal alloys comprising 30 to 70% of an alkali metal fluoborate, 30 to 70% of an alkali metal fluotitanate and 10 to 40% of sodium chloride.

2. A flux composition for treating aluminum and aluminum base metal alloys comprising 30 to 70% of an alkali metal fluoborate, 30 to 70% of an alkali metal fluotitanate and 10 to 40% of cryolite.

3. A flux composition for treating aluminum and aluminum base metal alloys comprising 30 to 70% of an alkali metal fluoborate, 30 to 70% of an alkali metal fluotitanate and 10 to 40% of calcium fluoride, at least one of said alkali metals being sodium.

4. A method of improving the characteristics of aluminum and aluminum base metal alloys, including heat-treatable alloys, comprising maintaining said aluminum and aluminum alloy in a molten state, and inserting within the body of said molten aluminum and aluminum alloy a treating mixture comprising an alkali metal fluoborate and an alkali metal fluotitanate, the alkali metal of at least one of said compounds being sodium, said combined alkali metal fluoborate and alkali metal fluotitanate being used in an amount of at least 0.1% by weight of the weight of the metal being treated.

5. A method of improving the characteristics of aluminum and aluminum-containing metals comprising maintaining said aluminum and aluminum-containing metals in a molten state while treating said metals with an intimate mixture of heat bonded ingredients comprising 25 to 75% of an alkali metal fluoborate and 25 to 75% of an alkali metal fluotitanate, at least one of said alkali metals being sodium, said combined alkali metal fluoborate and alkali metal fluotitanate being used in an amount of at least 0.1% by weight of the weight of the metal being treated.

6. A method of treating aluminum and aluminum base metals comprising melting said metal and inserting into the body of said molten metal and near the bottom thereof a compact fused mass of fluxing material containing 25

to 75% of an alkali fluoborate and 25 to 75% of an alkali fluotitanate at least one of said alkali metals being sodium, said combined alkali metal fluoborate and alkali metal fluotitanate being used in an amount of at least 0.1% by weight of the weight of the metal being treated.

7. A flux composition comprising 25 to 75% of an alkali metal fluoborate, 25 to 75% of an alkali metal fluotitanate, at least one of said alkali metals being sodium, and substantially the remainder of said composition being made up of at least one material of the group consisting of sodium chloride, sodium fluoride, calcium fluoride, sodium aluminum fluoride and magnesium fluoride.

8. The composition of claim 7 in which said alkali metal fluoborate and alkali metal fluotitanate are substantially anhydrous and are bonded together through the application of heat.

9. A flux composition comprising 25 to 75% of an alkali metal fluoborate and 25 to 75% of an alkali metal fluotitanate, at least one of said alkali metals being sodium.

10. A flux package for aluminum and aluminum base metal alloys comprising a compact fused mass containing 25 to 75% of an alkali metal fluoborate and 25 to 75% of an alkali metal fluotitanate, at least one of said alkali metals being sodium.

JAMES A. DAVIS.  
LA VERNE W. EASTWOOD.

References Cited in the file of this patent

UNITED STATES PATENTS

| Number    | Name               | Date          |
|-----------|--------------------|---------------|
| 1,596,888 | Pacz               | Aug. 24, 1926 |
| 1,636,881 | Tullis             | July 26, 1927 |
| 1,896,201 | Stern-Rainer       | Feb. 7, 1933  |
| 2,085,697 | Frost et al.       | June 29, 1937 |
| 2,447,672 | Smith, Jr., et al. | Aug. 24, 1948 |
| 2,497,119 | Fink               | Feb. 14, 1950 |

FOREIGN PATENTS

| Number  | Country       | Date          |
|---------|---------------|---------------|
| 456,462 | Great Britain | Nov. 10, 1936 |

OTHER REFERENCES

"American Foundryman," April 1947, page 123.